

Dec. 3, 1935.

J. O. WHITELEY

2,022,700

PIN FOR ARTIFICIAL TEETH AND METHOD OF PRODUCING SAME

Filed May 15, 1934



FIG. 1



FIG. 2



FIG. 3

FIG. 6



FIG. 4



FIG. 5

INVENTOR.

Joseph O. Whiteley.

By   
Attorney.

## UNITED STATES PATENT OFFICE

2,022,700

PIN FOR ARTIFICIAL TEETH AND METHOD  
OF PRODUCING SAMEJoseph O. Whiteley, York, Pa., assignor to The  
Dentists' Supply Company of New York, a cor-  
poration of New York

Application May 15, 1934, Serial No. 725,690

3 Claims. (Cl. 32—10)

The object of my invention is to provide an anchoring pin, for artificial teeth, which will be strong and durable in construction and include protection against deleterious effects due to oxidation and presence of acids in the oral fluids, and which also has capacity to prevent injury to the pin during various heat changes required in the manufacturing processes.

In carrying out the invention it is my primary purpose to construct a composite wire having a core of strong base metal and provided with one or more covering layers of precious metals or alloys thereof, the same being mechanically or physically applied to the core to form a close and dense structure which will be impervious to gases, acids and other destructive solutions, and adapted to being hammered, swaged, rolled or drawn into a fine wire, which is thereafter cut and shaped to form individual pins for artificial teeth; the said covering layer or layers being selected for their properties which are chemically inert to the base metal core and capable of withstanding frequent annealings during the wire producing process.

Still further, it is my intention to apply a precious metal covering layer to the pins after having been cut and formed from the drawn wire, which outer covering layer is electrolytically applied so as to fully cover both the head and shank portions of the pin, giving to it not only an ornamental finish which is self-retaining but also affording additional protection against injury to the pin when in use in a denture.

According to the invention, the dental pin comprises a base metal core with a jacket of densified precious metal chemically inert to the core covering all but the head, crown and foot of said pin, and a uniform outer covering of homogeneous precious metal completely encasing the pin. The pin is made by first mechanically applying a covering of precious metal to a base metal core, then compressing same into a fine wire, then cutting and shaping the densified wire into tooth pin forms, and finally covering the entire pin with an outer layer of precious metal.

The drawing illustrates an embodiment of the invention and the views therein are as follows:

Fig. 1 is a vertical sectional view of an artificial tooth with my improved pin forming a part thereof;

Fig. 2 is a side view of a base metal core structure mechanically or physically connected by solder or otherwise to a tubular sheath or hollow cylindrical covering of precious metal;

Fig. 3 is a longitudinal sectional view illustrating

ing a pin structure whose shank has been stretched or elongated and whose head has been upset, swaged and compressed, the same having a base metal core and a covering layer of precious metal;

Fig. 4 is a similar view to that shown in Fig. 3, but with an additional covering layer of non-corrodible precious metal which entirely covers the outer surface of the pin;

Fig. 5 is a cross-section of the pin taken on line 4—4 of Fig. 4; and

Fig. 6 is an enlarged sectional view of the head of the pin, to more clearly illustrate these covering structures.

Broadly considered, my improved pin embodies a structure comprising a base metal core 2, one or more mechanically imposed covering layers 3 of precious metal or a suitable alloy thereof, and which, after being properly shaped, is finally coated by an electrolytically deposited covering 4 of precious metal, preferably gold, which is especially resistant to oxidation and acids in the oral fluids.

In the production of my improved pin structure, I employ a strong base metal core 2, either of nickel, tantalum, tungsten and the like, which, while being relatively inexpensive and durable, are resistant to high temperatures. These metals have, however, a relatively low resistance or defense against oxidation and acids of the mouth, and hence must be protected by one or more covering layers of precious metals which will be resistant to such deleterious effects. Such covering layer may be of silver, gold, any metal of the platinum group, or a suitable alloy of the precious metals, such as would be included in an alloy of palladium and silver, and by my present method, is mechanically or physically applied to the base metal core.

The advantage of a mechanically or physically applied covering layer to the base metal core is that, due to being hammered, rolled, drawn, swaged or the like, the covering will have a dense close grain structure which is impervious to acid solutions and gases and provides the base metal core with a protecting covering, whereas a covering applied by electro-deposition would, through the crystalline character of the layer, be more or less porous and hence, if used alone, would fail as a protecting layer or covering for the base metal. For this reason, the use of a dense buffer layer in association with an electrolytically deposited layer will insure the physical protection of the pin, and the outer electrolytically deposited layer (preferably gold) will further assure the

- permanency of the desired external color and beauty of surface. Furthermore, the mechanically or physically imposed covering layer may be fairly thin, if so desired, thus reducing the cost and quantity of precious metals used in covering the base metal core, since the structure, according to my invention, is to be further protected by an electrolytically deposited covering of precious metals.
- 10 After the base metal core structure 2a has been mechanically or physically covered with one or more layers 3a of precious metals, it is then reduced by means of rolling, swaging and drawing, with frequent annealings, into a fine wire suitable for cutting and shaping into tooth pin forms for use with artificial teeth. Where mechanically applied layers only are used, the necessity of frequent annealings in reducing the thick wire to a fine wire has a tendency to cause the underlying base metal core to penetrate the precious metal covering and cause it to oxidize and discolor, and for this reason a fairly heavy covering of precious metal is necessary to resist the infiltration tendency of the metal of the underlying core where such mechanically applied layers only are used. Furthermore, in the cutting and shaping of the tooth pin forms from the fine wire, the covering layer 3 immediately outside of the base metal 2 is crowded inward in the upset portion to impart, to a more or less degree, a closure at both ends of the pin. This closure, however, while covering a part of the head and shank ends of the pin, leaves a portion of the base metal core 2 exposed in said parts, as indicated at 5 and 6, thus permitting injury to the pin when subjecting the same (while attached to an artificial tooth) to high temperatures in the manufacturing processes, and also allows the pin to be affected by gases, acids in the mouth, and other injurious effects while in use in a denture.
- To overcome these defects, I combine, with the mechanically applied layer, an electrolytically deposited or applied outer layer 4 of precious metals, such as silver, gold, any of the platinum group metals, or suitable alloys of these metals, to the pin structure. By combining a mechanical and an electrolytically applied covering to the base metal core, the mechanical covering may be selected, because of its properties, to act as a chemical buffer between the core and the electrolytically applied covering, and by reason of which will prevent the formation of a gold-nickel eutectic. For example, in the case of a tooth pin with a nickel core and a pure gold covering, I find that under heat the nickel and gold have an affinity for each other, such that the nickel will alloy with and discolor the gold at a temperature lower than the melting point of either metal. Gold and nickel form a eutectic or melting point around 1700° to 1800° F. Therefore, in the case of a nickel pin with a single mechanically applied gold covering, the gold covering must be relatively thick, which is expensive. In my present method, I employ inner and outer coverings or layers of precious metals, both of which may be relatively thin, thus considerably reducing the cost and quantity of precious metals necessary to form such coverings or layers.
- 70 Furthermore, because of the combination mechanically applied inner layer and electrolytically deposited outer layer, certain advantages are obtained; for example, the outer layer need not be subjected to the frequent annealing temperatures necessary when applying the mechani-

cal layer of precious metal to the core, or when working down the bar or structure as in the manufacture of wire; because such repeated annealing heats would require the coverings to be fairly heavy in order to avoid the tendency of the underlying metal to infiltrate the covering and discolor its surface. Further, by electrolytically depositing the outer covering over the mechanically applied layer, the extreme head and shank ends of the pin are completely covered with the protective layer of precious metal, as shown at 5a and 6a in Fig. 4, which not only greatly adds to the protection of the pin against deleterious effects and insolubility in oral solutions, but also gives to the pin an ornamental covering of desirable color and surface beauty.

Heretofore, in the method of making mechanically plated articles, such as tooth pins, the method was as follows: A nickel bar is covered mechanically with a layer of silver and then mechanically again covered with an outer layer of gold. The gold in such a case was quite thick in order to resist the tendency of the silver layer to penetrate and blanch its color when heated. When a wire so constructed was reduced and tooth pins cut therefrom, a spot of nickel was exposed on the head and shank ends of the pin. In my improved method, these objections are entirely overcome and a tooth pin is produced which will withstand not only deleterious effects due to oxidation and acids in the oral fluids, but is completely covered from head to shank end with a covering of precious metal of desirable color. According to my improved method, I first cover the base metal bar with a mechanically applied layer or layers of precious metal or a suitable alloy thereof, selecting a metal which will be chemically inert to the core metal and which has the properties desired for the particular application and use to which the bar is subjected; I then work the bar into a fine wire by rolling or drawing; and thereafter cut and form the wire into tooth pins. The formed pins are then electro-plated or gilded with a precious metal of desirable color and chemical properties to thoroughly protect the pins against gases and oral fluids. The pin thus made is therefore provided with a uniform outer covering of homogeneous precious metal completely encasing the pin. A tooth pin so constructed has every desirable advantage over pins constructed under the old method; and in addition is relatively inexpensive, as both the inner and outer coverings may be thin; repeated applications of heat necessary to work down the bar into a fine wire structure are avoided; the entire pin from head to shank ends is completely covered with a protective layer of precious metal; and the completed pin presents an ornamental finish of desirable color and surface beauty fully protected against deleterious effects and insolubility in oral solutions.

Of course the tooth pins shown and described herein may be modified in various ways without departing from the invention herein set forth and hereafter claimed.

I claim:

1. A pin for artificial teeth, comprising a base metal core, a jacket of densified precious metal chemically inert to the core and covering all but the head crown and foot of said pin, and a uniform outer covering of homogeneous precious metal completely encasing the pin.

2. The herein described method of making a pin for artificial teeth, comprising the steps of

first mechanically applying a covering of precious metal to a base metal core, then compressing same into a fine wire, then cutting and shaping the densified wire into tooth pin forms, and finally covering the entire pin with an outer layer of precious metal.

3. The herein described method of making a pin for artificial teeth, which consists in mechan-

ically applying a covering of precious metal to a base metal core and compressing the same into a fine wire, thereafter cutting and shaping the densified wire into tooth pin forms, and finally electrolytically depositing upon the entire surface of the tooth pin forms an outer covering or layer of precious metal.

JOSEPH O. WHITELEY.